

## 1

3,274,080

 BRIGHTENERS AND PROCESS FOR CYANIDE  
ZINC ELECTRODEPOSITION

Robert E. Harrover, Jr., North Huntingdon Township, Westmoreland County, Pa., assignor, by mesne assignments, to Cowles Chemical Company, Shaker Heights, Ohio, a corporation of Ohio

No Drawing. Filed May 25, 1962, Ser. No. 197,598  
17 Claims. (Cl. 204—55)

This invention relates to bright zinc electroplating methods, novel brightener addition compositions and novel electrolyte compositions.

The typical electrodeposits from an aqueous cyanide zinc electrolyte are dull and granular. Numerous attempts have been made by those working in the art to improve the character of zinc deposits obtained from aqueous alkaline cyanide baths. Many addition agents have been used and some progress has been made. Nonetheless, electrodeposits of zinc from aqueous cyanide plating baths typically lack one or more desirable properties such as brightness, grain refinement and attractive color, or for example the bath may lack good throwing power.

Accordingly, it is the general object of this invention to provide novel brightener addition agents or compositions, novel aqueous alkaline cyanide zinc electrolyte compositions with good throwing power and plating methods which will enable the attainment of bright, fine grained and attractive zinc deposits.

It is a more particular object of this invention to provide a particular combination of additives which can be effectively employed in an aqueous alkaline cyanide zinc bath to produce superior bright, ductile zinc coatings.

A further object of this invention is to provide novel electrolyte compositions which will produce superior bright, fine grained, smooth zinc coatings and which exhibit excellent throwing power so that a uniform bright zinc coating may be deposited on irregularly shaped and recessed objects.

Still another object of this invention is to provide a zinc electrodeposit which responds in an excellent manner to clear conversion coatings and dilute oxidizing bright dips.

Briefly, the present invention accomplishes the above cited objects by providing a class of compounds which provide a beneficial effect on the brightness and color of zinc electrodeposits when employed in an aqueous alkaline zinc cyanide electrolyte. Moreover, these compounds and others, when employed in combination with polyvinyl alcohol, exert a profound and synergistic effect upon the brightness, color and smoothness of the resulting zinc plate.

Further objects and advantages of the invention will become apparent as the following description proceeds and features of novelty which characterize the invention will be pointed out in particularity in the claims annexed to and forming a part of this specification.

It has now been found that a particular class of compounds can be used to produce an improved zinc electrodeposit from aqueous alkaline cyanide electrolytes. When added to an aqueous alkaline zinc cyanide electrolyte, at least one brightener compound selected from the group consisting of compounds having the formulas:

(1)



and

(2)



## 2

where R is selected from the group consisting of monovalent and divalent saturated substituted and unsubstituted hydrocarbon radicals having from 1 to 4 carbon atoms and the substituents are selected from the group consisting of —NH<sub>2</sub>, —OH and —COOR<sub>1</sub>, said R<sub>1</sub> is selected from the group consisting of H, NH<sub>4</sub> and alkali metal salts, M is selected from the group of monovalent and divalent materials consisting of NH<sub>4</sub>, CH<sub>3</sub>NH<sub>3</sub>, (CH<sub>3</sub>)<sub>2</sub>NH<sub>2</sub>, Na, K, Ca, Zn, Mg, Cd, Ni, Fe, Co, Mo and Mn and n is equal to the valence of M, will produce an electrodeposit with improved brightness and grain size, especially at low current densities, as for example 1/2 to about 15 ampere/ft.<sup>2</sup>.

These compounds may be incorporated into aqueous alkaline cyanide zinc plating baths as illustrated by the following specific examples, with the indicated results.

## Example I

|                             | Oz./gal. |
|-----------------------------|----------|
| Zinc oxide                  | 5.6      |
| Sodium cyanide              | 12.3     |
| Sodium hydroxide            | 5.0      |
| Tetraethylthiuram disulfide | 0.02     |

Zinc may be electrodeposited from this electrolyte with an improvement in the brightness of the deposit, particularly in the range of 1/2 to 15 amperes/ft.<sup>2</sup>.

## Example II

|                             | Oz./gal. |
|-----------------------------|----------|
| Zinc oxide                  | 5.6      |
| Sodium cyanide              | 10.5     |
| Sodium hydroxide            | 3.4      |
| Dibutylidithiuram disulfide | 0.006    |

Zinc may be electrodeposited from this electrolyte with an improvement in the brightness and grain size of the deposit.

## Example III

|                                           | Oz./gal. |
|-------------------------------------------|----------|
| Zinc oxide                                | 5.6      |
| Sodium cyanide                            | 12.3     |
| Sodium hydroxide                          | 5.0      |
| Trimethyl-N-acetic acid thiuram disulfide | 0.01     |

Zinc may be electrodeposited from this electrolyte with an improvement in the brightness of the deposit, particularly in the range of 1 to 10 amperes/ft.<sup>2</sup>.

## Example IV

|                                              | Oz./gal. |
|----------------------------------------------|----------|
| Zinc oxide                                   | 5.0      |
| Sodium cyanide                               | 12.0     |
| Sodium hydroxide                             | 5.0      |
| Trimethyl-N-sodium acetate thiuram disulfide | 0.03     |

Zinc may be electrodeposited from this electrolyte with an improvement in the brightness of the deposit, particularly in the range of 1/2 to 18 amperes/ft.<sup>2</sup>.

## Example V

|                                                | Oz./gal. |
|------------------------------------------------|----------|
| Zinc oxide                                     | 5.6      |
| Sodium cyanide                                 | 12.3     |
| Sodium hydroxide                               | 5.0      |
| Trimethyl-N-ammonium acetate thiuram disulfide | 0.003    |

Zinc may be electrodeposited from this electrolyte with a visible improvement in brightness and grain size.

## Example VI

|                              | Oz./gal. |
|------------------------------|----------|
| Zinc oxide                   | 5.6      |
| Sodium cyanide               | 12.3     |
| Sodium hydroxide             | 5.0      |
| Zinc dimethyldithiocarbamate | 0.05     |

Zinc may be electrodeposited from this electrolyte with a significant improvement in brightness and grain size.

*Example VII*

|                                  | Oz./gal. |
|----------------------------------|----------|
| Zinc oxide                       | 5.6      |
| Sodium cyanide                   | 12.3     |
| Sodium hydroxide                 | 5.0      |
| Nickel dimethyloldithiocarbamate | 0.01     |

Zinc may be electrodeposited from this electrolyte with an improvement in the brightness and grain size of the deposit, particularly in the range of  $\frac{1}{2}$  to 10 amperes/ft.<sup>2</sup>.

*Example VIII*

|                                                | Oz./gal. |
|------------------------------------------------|----------|
| Zinc oxide                                     | 5.6      |
| Sodium cyanide                                 | 12.3     |
| Sodium hydroxide                               | 5.0      |
| Sodium methyl-N-sodium acetate dithiocarbamate | 0.008    |

Zinc may be electrodeposited from this electrolyte with an improvement in the brightness and grain size of the deposit, particularly in the range of  $\frac{1}{2}$  to 10 amperes/ft.<sup>2</sup>.

It is to be understood that the foregoing examples are only illustrative and that other compounds within the class defined by the structural formulas presented hereinabove may be employed according to this invention. For example, potassium, calcium, magnesium, cadmium, cobalt, molybdenum and manganese compounds may be substituted for the zinc, nickel and sodium compounds of the foregoing specific examples, with equivalent results.

The compounds may be employed in concentrations limited only by their solubility in the aqueous alkaline zinc cyanide bath. However, it is preferred to maintain the concentration in a range of from about 0.003 to about 0.02 oz./gal. for optimum results.

The use of polyvinyl alcohol as a brightener addition agent for zinc cyanide plating baths is known and has been so described in the prior art. However, it has now been discovered that when polyvinyl alcohol is employed in combination with at least one of any of the compounds described heretofore, hereinafter referred to as dithiocarbamate compounds, a profound effect on the brightness of the zinc deposit is produced. The combination also surprisingly increases the throwing power of the bath so that uniform bright zinc coatings may be deposited on irregularly shaped and recessed objects. The combination produces a much brighter, more uniform zinc deposit over a wider current density range than when either material is used alone.

Also known and described in the art as brightener addition agents for zinc cyanide plating baths are the reaction products obtained by reacting substantially equimolar quantities of at least one compound having the nucleus



with ammonia or certain derivatives thereof as will be described more fully hereinbelow. The preparation of these reaction products, among others, are described in U.S. Patent 3,018,232, assigned to the assignee of this invention.

It has been discovered that when at least one of the reaction products described hereinbelow is employed in combination with polyvinyl alcohol, a profound effect on the brightness and grain refinement of the zinc is produced, similar to the effect of employing polyvinyl alcohol in combination with the described dithiocarbamate compounds.

*Examples of compounds having the nucleus*



for the purposes of this invention, are 2-thiohydantoin and substitution derivatives of 2-thiohydantoin having at

least one organic substituent in the 1, 5 positions. The nucleus of these 2-thiohydantoin substitution derivatives has the following structure:



10 Various organic radicals may be substituted at one or both of the 1 or 5 positions, providing the compound obtained upon reaction with ammonia or derivatives thereof is soluble in the aqueous alkaline zinc cyanide electrolyte in an amount sufficient to produce an appreciable improvement in brightness and smoothness of the zinc deposited. Examples of suitable compounds are:

- 2-thiohydantoin  
1-acetyl-2-thiohydantoin  
5 (2-hydroxylbenzal)-2-thiohydantoin  
5-furfural-2-thiohydantoin  
5-benzal-2-thiohydantoin  
1-methyl-2-thiohydantoin

25 Other examples of compounds having the nucleus



which are suitable for reaction with ammonia or derivatives thereof to produce the reaction products employed 30 in this invention include:

- 2-thiobarbituric acid  
1-acetyl-2-thiobarbituric acid  
1-benzoyl-2-thiobarbituric acid  
1,5-diacyetyl-2-thiobarbituric acid  
35 2-thiopyrrolidone-4  
5-thio-1,2,4-trazolidinone-3  
4-thioxazolidinone-4  
4-thiothiazolidinone-4  
3-thio-1,2,4-oxadiazolidinone-5  
3-thio-1,2,4-thiadiazolidinone-5  
2-thioazolidinone-6  
40 2-thio-1,3-diazolidinone-4  
2-thio-1,4-diazolidinone-6  
3-thio-1,2,4-triazolidinone-5  
45 2-thio-1,3,5-triazolidinone-4  
5-thio-1,2,4-triazolidinone-3  
1-thio-2-benzazolone-3  
3-thio-2-benzazolone-1

50 Reaction products suitable for use in this invention, may be produced by reacting the compounds having the nucleus



55 heretofore described, with compounds having the formula



60 wherein R is a radical selected from the group consisting of hydrogen; monovalent and divalent saturated substituted and unsubstituted aliphatic hydrocarbon radicals having from 1 to 4 carbon atoms in which the substituents are selected from the group consisting of  $-\text{NH}_2$  and  $-\text{OH}$  radicals, phenyl radicals, monovalent and divalent alicyclic radicals containing from 5 to 6 carbon atoms in the ring in which the substituents are selected from the group consisting of  $-\text{CH}_3$ ,  $-\text{NH}_2$  and  $-\text{OH}$  radicals and aminophenyl radicals.

65 Specific examples of the amine compounds included within the scope of the terms identified above include:

- ammonia  
isopropylamine

monoethanolamine  
ethylenediamine  
dibutylamine  
methylethylolamine  
diisopropanolamine  
methyl-propylenediamine  
diethylenediamine  
propylolmethylenediamine  
cyclopentylamine  
dicyclohexylamine  
cyclopentylmethylamine  
cyclohexylisopropylolamine  
cyclopentylethylenediamine  
3-methylcyclohexylamine  
1,2-diaminocyclopentane  
4-hydroxycyclohexylamine  
aniline  
p-aminoaniline  
methylaniline  
ethyl-4-methylcyclohexylamine  
4-methylaminocyclohexylamine  
1-methylamino-2-hydroxycyclopentane  
p-aminomethylaniline  
cyclohexylaniline  
diphenylamine  
2-methylhexylethylolamine  
N-ethylolaniine  
phenyl-4-aminocyclohexylamine  
N-ethylol-p-aminoaniline  
4-methylcyclohexylpropylenediamine  
dimethylcyclohexylamine  
phenylethylenediamine  
di-4-aminocyclohexylamine  
N-cyclopentylaminoaniline  
3-isopropylaminocyclohexanol  
ethylol-1,4-diaminocyclohexane  
phenylcyclohexanolamine  
phenyl-p-aminoaniline  
N-(2'-aminoethylene)-1,4-diaminocyclohexane  
N-(2'-aminoisopropylene)-4-aminocyclohexanol  
N-cyclopentyl-1,4-diaminocyclohexane  
cyclohexylmethylcyclohexylamine  
di-p-aminophenylamine  
p-aminophenyl-4-methylcyclohexylamine  
4-methylcyclohexylphenylamine  
p-amino-phenylethylenediamine  
p-aminophenyl-3-aminocyclopentylamine  
N-(3'-hydroxycyclohexyl)-p-aminoaniline  
4-cyclohexylaminocyclopentanol-3  
N-(3'-methylcyclopentyl)-1,4-diaminocyclohexane  
4,4'-dicyclohexaneolylamine  
N-(3'-methylcyclohexyl)-4-aminocyclohexane  
N-(2'-hydroxycyclohexyl)-1,4-diaminocyclohexane

The preparation of the reaction product compounds discussed hereinabove as suitable for addition to aqueous alkaline cyanide zinc plating baths in accordance with the present invention, is also disclosed in U.S. Patent No. 2,972,572 issued to R. P. Cope, Jr., et al. and assigned to the assignee of the present invention. It will be understood that substantially equimolar quantities actually take part in the reaction although other stoichiometry may be employed with less efficiency.

The polyvinyl alcohol for use in this invention may be partially acetylated. It is preferred that the polyvinyl alcohol be about 20-40% acetylated for ease of solubility in the resultant additive mixture. Low residual acetate polyvinyl alcohol resins require temperatures of 85-95° C. (185-203° F.) to prepare resin solutions. A low molecular weight resin is also preferred for ease and completeness of solution. This does not limit the kind of polyvinyl alcohol resin which may be used but only sets forth the preferred resin for this invention. It should be understood that the type or molecular weight of the polyvinyl alcohol is limited only by the solubility

5 in the aqueous alkaline zinc cyanide electrolyte. The polyvinyl alcohol employed must, of course, be soluble in the electrolyte. The polyvinyl alcohol may be used in combination with at least one reaction product or di-5 thiocarbamate compound or with at least one reaction product and dithiocarbamate compound.

10 The combination of polyvinyl alcohol with either the reaction product or dithiocarbamate compound, or with both, is incorporated into aqueous alkaline zinc cyanide 10 plating baths as illustrated by the following specific examples:

*Example IX*

|                                                    | Oz./gal. |
|----------------------------------------------------|----------|
| Zinc oxide                                         | 5.6      |
| 15 Sodium cyanide                                  | 10.5     |
| Sodium hydroxide                                   | 3.0      |
| Polyvinyl alcohol                                  | 0.1      |
| Reaction product of 2-thiohydantoin<br>and ammonia | 0.01     |

20 Bright zinc may be electrodeposited from this electrolyte in the range of from about 5 to about 50 amperes/ft.<sup>2</sup>. The plating will be semi-bright in the range of about 50 to about 90 amperes/ft.<sup>2</sup>. The color of the deposit will be whiter and more pleasing in appearance than the normal yellowish color.

*Example X*

|                                                                                                                                                                                                       | Oz./gal. |
|-------------------------------------------------------------------------------------------------------------------------------------------------------------------------------------------------------|----------|
| Zinc oxide                                                                                                                                                                                            | 5.6      |
| 30 Sodium cyanide                                                                                                                                                                                     | 12.3     |
| Sodium hydroxide                                                                                                                                                                                      | 5.0      |
| Polyvinyl alcohol                                                                                                                                                                                     | 0.025    |
| Zinc dibutylthiocarbamate                                                                                                                                                                             | 0.01     |
| 35 Bright zinc may be electrodeposited in the range of from about 2 to about 28 amperes/ft. <sup>2</sup> . A deposit more reflective than normal will be apparent above 28 amperes/ft. <sup>2</sup> . |          |

*Example XI*

|                                                               | Oz./gal. |
|---------------------------------------------------------------|----------|
| Zinc oxide                                                    | 5.6      |
| Sodium cyanide                                                | 12.3     |
| Sodium hydroxide                                              | 5.0      |
| Polyvinyl alcohol                                             | 0.05     |
| 45 Reaction product of 2-thiohydantion and 2-<br>aminoethanol | 0.1      |

Bright zinc may be electrodeposited from this electrolyte in the range of from about 5 to about 50 amperes/ft.<sup>2</sup>.  
50 The plating will be semi-bright in the range of about 50 to about 90 amperes/ft.<sup>2</sup>. The color of the deposit will be whiter and more pleasing in appearance than the normal yellowish color.

*Example XII*

|                              | Oz./gal. |
|------------------------------|----------|
| Zinc oxide                   | 5.6      |
| Sodium cyanide               | 12.3     |
| Sodium hydroxide             | 5.0      |
| 60 Polyvinyl alcohol         | 0.025    |
| Zinc dimethyldithiocarbamate | 0.1      |

Bright zinc may be electrodeposited in the range of from about 2 to about 28 amperes/ft.<sup>2</sup>. A deposit more reflective than normal will be apparent above 28 amperes/ft.<sup>2</sup>.

*Example XIII*

|                                                             | Oz./gal. |
|-------------------------------------------------------------|----------|
| Zinc oxide                                                  | 5.6      |
| 70 Sodium cyanide                                           | 12.3     |
| Sodium hydroxide                                            | 5.0      |
| Polyvinyl alcohol                                           | 0.004    |
| Tetrapropylthiuramdisulfide                                 | 0.006    |
| Reaction product of 1-acetyl-2-thiohydantoin and<br>aniline | 0.008    |

Zinc that is bright and fair in color may be electro-deposited from this electrolyte.

Example XIV

|                                                         | Oz./gal. |
|---------------------------------------------------------|----------|
| Zinc oxide                                              | 5.0      |
| Sodium cyanide                                          | 12.0     |
| Sodium hydroxide                                        | 5.0      |
| Polyvinyl alcohol                                       | 0.08     |
| Zinc dimethyldithiocarbamate                            | 0.02     |
| Reaction product of 2-thiohydantoin and 2-amino-ethanol | 0.3      |

Zinc that is very bright with good color may be electro-deposited from this electrolyte. The brightness on the extreme low current density range will be particularly outstanding.

It is to be understood that the concentration of the brightening agents, either singly or in combination, is limited only by the solubility of the agents in the aqueous alkaline zinc cyanide plating bath. It is preferred that a minimum concentration of 0.0005 oz./gal. of each agent added be maintained in the bath. As an upper limit, it is preferred that the maximum concentration of the reaction products be about 0.5 oz./gal. and that the concentration of polyvinyl alcohol be limited to a maximum of about 0.1 oz./gal. In the preferred electrolyte composition, the dithiocarbamate compounds may be employed up to the limit of solubility.

The electrolyte may be conveniently prepared by adding a novel addition agent brightener composition comprising (A) polyvinyl alcohol and (B) the reaction product compound obtained by reacting substantially equimolar quantities of at least one compound having the nucleus



with at least one compound selected from the group consisting of compounds having the formula



wherein R is a radical selected from the group consisting of hydrogen, monovalent and divalent saturated substituted and unsubstituted aliphatic hydrocarbon radicals having from 1 to 4 carbon atoms in which the substituents for the substituted hydrocarbon radicals are selected from the group consisting of  $-\text{NH}_2$  and  $-\text{OH}$  radicals, phenyl radicals, monovalent and divalent alicyclic radicals containing from 5 to 6 carbon atoms in the ring in which the substituents are selected from the group consisting of  $-\text{CH}_3$ ,  $-\text{NH}_2$ ,  $-\text{OH}$  radicals and aminophenyl radicals to an aqueous alkaline zinc cyanide plating bath prepared according to principles known in the art. For example, an addition agent brightener composition comprising (A) polyvinyl alcohol and (B) the reaction product compound obtained by reacting substantially equimolar quantities of the 2-thiohydantoin and 2-aminoethanol may be added to an aqueous alkaline zinc cyanide electrolyte to provide the concentrations described hereinabove.

An electrolyte may also be prepared by adding a novel addition agent brightener composition comprising (A) polyvinyl alcohol and (B) at least one dithiocarbamate compound selected from the group consisting of compounds having the formulas



and



where R is selected from the group consisting of monovalent and divalent saturated hydrocarbon radicals having from 1 to 4 carbon atoms and in which the substituents are selected from the group consisting of  $-\text{NH}_2$ ,  $-\text{OH}$  and  $-\text{COOR}_1$ , said R<sub>1</sub> is selected from the group consisting of H, NH<sub>4</sub> and alkali metal salts, M is selected from the group of monovalent and divalent materials consisting of NH<sub>4</sub>, CH<sub>3</sub>NH<sub>3</sub>, (CH<sub>3</sub>)<sub>2</sub>NH<sub>2</sub>, Na, K, Ca, Zn, Mg, Cd, Ni, Fe, Co, Mo and Mn and n is equal to the valence of M, to known aqueous alkaline zinc cyanide plating baths. For example, an addition agent composition comprising (A) polyvinyl alcohol and (B) zinc dimethyldithiocarbamate may be added to an aqueous alkaline zinc cyanide bath to obtain the desired electrolyte.

An electrolyte may also be prepared by adding a novel addition agent composition, comprising (A) polyvinyl alcohol, (B) at least one described reaction product compound and (C) at least one described dithiocarbamate compound to known aqueous alkaline zinc cyanide electrolytes.

For example, the novel composition comprising (A) polyvinyl alcohol, (B) a brightener compound obtained by reacting substantially equimolar quantities of 2-thiohydantoin and 2-aminoethanol and (C) zinc dimethyldithiocarbamate may be added to an aqueous alkaline zinc cyanide plating bath to obtain an electrolyte of this invention.

The electrodeposit produced with an aqueous alkaline zinc cyanide electrolyte containing polyvinyl alcohol together with either one or both of the reaction product compounds and dithiocarbamate compounds responds in an excellent manner to clear conversion coatings and dilute oxidizing bright dips. When subjected to a ten second dip in a clear conversion coating bath the deposits became brilliant and exhibited a pleasing blue white color.

It is to be understood that the zinc oxide, sodium cyanide and sodium hydroxide contents of the cyanide baths outlined hereinabove are only examples and that applicant's invention is not to be limited by these specific cyanide bath compositions. For example, zinc cyanide may be employed in place of zinc oxide with an appropriate reduction in the sodium cyanide content so that a proper cyanide-zinc ratio may be maintained. Other aqueous alkaline zinc cyanide compositions are known in the art and may be employed with the addition agent compositions of this invention.

While there have been shown and described what are presently considered to be the preferred embodiments of the invention, modifications thereto will readily occur to those skilled in the art. It is not desired, therefore, that the invention be limited to the specific methods and compositions shown and described and it is intended to cover in the appended claims all such modifications as fall within the true spirit and scope of the invention.

I claim as my invention:

1. An aqueous alkaline zinc cyanide plating solution for electrodepositing zinc containing zinc ions and at least one brightener compound selected from the group consisting of compounds having the formulas



and



where R is selected from the group consisting of monovalent and divalent saturated substituted and unsubstituted hydrocarbon radicals having from 1 to 4 carbon atoms.

atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M.

2. An aqueous alkaline zinc cyanide plating solution for electrodepositing zinc containing zinc ions and at least one brightener compound selected from the group consisting of compounds having the formulas



and



where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M, said brightener being present in a concentration of at least 0.0005 ounces per gallon.

3. An aqueous alkaline zinc cyanide plating solution for electrodepositing zinc containing zinc ions and at least one brightener compound selected from the group consisting of compounds having the formulas



and



where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M, said brightener being present in a concentration range of 0.003 to about 0.02 ounces per gallon.

4. An aqueous alkaline zinc cyanide plating solution for electrodepositing zinc containing zinc ions and tetramethylthiuramdisulfide in a concentration of at least 0.0005 ounces per gallon.

5. An aqueous alkaline zinc cyanide plating solution for electrodepositing zinc containing zinc ions and zinc dimethyldithiocarbamate in a concentration range of about 0.003 to about 0.02 ounces per gallon.

6. An aqueous alkaline zinc cyanide plating solution for electrodepositing zinc containing zinc ions, polyvinyl alcohol and at least one brightener compound selected from the group consisting of compounds having the formulas



and

(2)



where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M, said polyvinyl alcohol present in a concentration up to about 0.08 ounces per gallon and said brightener compound being present in a concentration of at least 0.0005 ounces per gallon.

7. An aqueous alkaline zinc cyanide plating solution for electrodepositing zinc containing zinc ions, polyvinyl alcohol and at least one brightener compound selected from the group consisting of compounds having the formulas



and



where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ ,  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,

$(\text{CH}_3)_2\text{NH}_2$ , Na, K, Ca, Zn, Mg, Cd, Ni, Fe, Co, Mo and Mn and n is equal to the valence of M, said polyvinyl alcohol present in a concentration up to about 0.08 ounce per gallon and said brightener compound being present in a concentration range of 0.003 to about 0.02 ounce per gallon.

8. An aqueous alkaline zinc cyanide plating solution for electrodepositing zinc containing zinc ions, (A) polyvinyl alcohol, (B) a brightener compound obtained by reacting substantially equimolar quantities of at least one compound having the nucleus



with at least one compound selected from the group consisting of compounds having the formula



wherein R is a radical selected from the group consisting of hydrogen, monovalent and divalent saturated substituted and unsubstituted aliphatic hydrocarbon radicals having from 1 to 4 carbon atoms in which the substituents for the substituted hydrocarbon radicals are selected from the group consisting of  $-\text{NH}_2$  and  $-\text{OH}$  radicals, monovalent and divalent alicyclic radicals containing from 5 to 6 carbon atoms in the ring in which the substituents are selected from the group consisting of  $-\text{CH}_3$ ,  $-\text{NH}_2$  and  $-\text{OH}$  radicals, phenyl radicals and aminophenyl radicals and (C) at least one brightener compound se-

lected from the group consisting of compounds having the formulas

(1)



and

(2)



where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials selected from the group consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M, said (A) present in a concentration up to about 0.08 ounce per gallon, said (B) present in a concentration of from 0.0005 to about 0.5 ounce per gallon and said (C) present in a concentration of at least 0.0005 ounce per gallon.

9. An addition agent composition suitable for introduction into an aqueous alkaline zinc cyanide electrolyte consisting essentially of (A) polyvinyl alcohol and (B) at least one brightener compound selected from the group consisting of compounds having the formulas

(1)



and

(2)



where R is selected from the group consisting of monovalent and divalent saturated hydrocarbon radicals having from 1 to 4 carbon atoms and in which the substituents are selected from the group consisting of  $-\text{NH}_2$ ,  $-\text{OH}$  and  $-\text{COOR}_1$  and  $\text{R}_1$  is selected from the group consisting of N,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, Mo and Mn and n is equal to the valence of M.

10. An addition agent composition suitable for introduction into an aqueous alkaline zinc cyanide electrolyte consisting essentially of (A) polyvinyl alcohol, (B) a brightener compound obtained by reacting substantially equimolar quantities of at least one compound having the nucleus



with at least one compound selected from the group consisting of compounds having the formula



wherein R is a radical selected from the group consisting of hydrogen, monovalent and divalent saturated substituted and unsubstituted aliphatic hydrocarbon radicals having from 1 to 4 carbon atoms in which the substituents for the substituted hydrocarbon radicals are selected from the group consisting of  $-\text{NH}_2$  and  $-\text{OH}$  radicals, monovalent and divalent alicyclic radicals containing from 5 to 6 carbon atoms in the ring in which the substituents

are selected from the group consisting of  $-\text{CH}_3$ ,  $-\text{NH}_2$  and  $-\text{OH}$  radicals, phenyl radicals and aminophenyl radicals and (C) at least one brightener compound selected from the group consisting of compounds having the formulas

5

(1)



10 and

(2)



15

where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials selected from the group consisting of  $\text{NH}_4$ ,  $\text{CH}_3\text{NH}_3$ ,  $(\text{CH}_3)_2\text{NH}_2$ , Na, K, Ca, Zn, Mg, Cd, Ni, Fe, Co, M and Mn and n is equal to the valence of M.

11. An addition agent composition suitable for introduction into an aqueous alkaline zinc cyanide electrolyte consisting essentially of (A) polyvinyl alcohol, (B) a brightener compound obtained by reacting substantially equimolar quantities of 2-thiohydantoin and 2-aminoethanol and (C) zinc dimethylthiocarbamate.

12. An addition agent composition suitable for introduction into an aqueous alkaline zinc cyanide electrolyte consisting essentially of (A) polyvinyl alcohol, (B) a brightener compound obtained by reacting substantially equimolar quantities of 2-thiobarbituric acid and aniline and (C) nickel diisopropylthiocarbamate.

13. An addition agent composition suitable for introduction into an aqueous alkaline zinc cyanide electrolyte consisting essentially of (A) polyvinyl alcohol (B) a brightener compound obtained by reacting substantially equimolar quantities of 1-acetyl-2-thiohydantoin and diisopropyl amine and (C) tetraethylthiuram disulfide.

14. A method of electrodepositing bright zinc metal comprising the steps of passing a current from an anode to a cathode to be plated in an aqueous alkaline zinc cyanide electrolyte containing zinc ions and at least one brightener compound selected from the group consisting of compounds having the formulas

50

(1)



55 and

(2)



60

where R is selected from the group consisting of monovalent and divalent saturated substituted and unsubstituted hydrocarbon radicals having from 1 to 4 carbon atoms and the substituents are selected from the group consisting of  $-\text{NH}_2$ ,  $-\text{OH}$  and  $-\text{COOR}_1$ , and  $\text{R}_1$  is selected from the group consisting of H,  $\text{NH}_4$  and alkali metal salts, M is selected from the group of monovalent and divalent materials consisting of  $\text{NH}_4$ ,  $\text{CH}_3\text{NH}_3$ ,  $(\text{CH}_3)_2\text{NH}_2$

70 Na, K, Ca, Zn, Mg, Cd, Ni, Fe, Co, Mo and Mn and n is equal to the valence of M.

15. A method of electrodepositing bright zinc metal comprising the steps of passing a current from an anode to a cathode to be plated in an aqueous alkaline zinc cyanide electrolyte containing zinc ions and (A) poly-

vinyl alcohol, (B) a brightener compound obtained by reacting substantially equimolar quantities of at least one compound having the nucleus



with at least one compound selected from the group consisting of compounds having the formula



wherein R is a radical selected from the group consisting of hydrogen, monovalent and divalent saturated substituted and unsubstituted aliphatic hydrocarbon radicals having from 1 to 4 carbon atoms in which the substituents for the substituted hydrocarbon radicals are selected from the group consisting of  $-NH_2$  and  $-OH$  radicals, monovalent and divalent alicyclic radicals containing from 5 to 6 carbon atoms in the ring in which the substituents are selected from the group consisting of  $-CH_3$ ,  $-NH_2$  and  $-OH$  radicals, phenyl radicals and aminophenyl radicals and (C) at least one brightener compound selected from the group consisting of compounds having the formulas



and



where R is selected from the group consisting of monovalent and divalent saturated substituted and unsubstituted hydrocarbon radicals having from 1 to 4 carbon atoms and the substituents are selected from the group consisting of  $-NH_2$ ,  $-OH$  and  $-COOR_1$ , and  $R_1$  is selected from the group consisting of H,  $NH_4$  and alkali metal salts, M is selected from the group of monovalent and divalent materials selected from the group consisting of  $NH_4$ ,  $CH_3NH_3$ ,  $(CH_3)_2NH_2$ , Na, K, Ca, Zn, Mg, Cd, Ni, Fe, Co, Mo and Mn and n is equal to the valence of M, said (A) present in a concentration up to about 0.08 ounce per gallon, said (B) present in a concentration of from 0.005 to about 0.5 ounce per gallon and said (C) present in a concentration of at least 0.0005 ounce per gallon.

16. An aqueous alkaline zinc cyanide plating solution for electrodepositing zinc containing zinc ions and at least one brightener compound selected from the group consisting of compounds having the formula

5



where R is selected from the group consisting of monovalent and divalent saturated substituted and unsubstituted hydrocarbon radicals having from 1 to 4 carbon atoms and the substituents are selected from the group consisting of  $-NH_2$ ,  $-OH$  and  $-COOR_1$ , and  $R_1$  is selected from the group consisting of H,  $NH_4$  and alkali metal salts.

17. An aqueous alkaline zinc cyanide plating solution for electrodepositing zinc containing zinc ions and at least one brightener compound selected from the group consisting of compounds having the formula

20



wherein R is selected from the group consisting of monovalent and divalent saturated substituted and unsubstituted hydrocarbon radicals having from 1 to 4 carbon atoms and the substituents are selected from the group consisting of  $-NH_2$ ,  $-OH$  and  $-COOR_1$ , and  $R_1$  is selected from the group consisting of H,  $NH_4$  and alkali metal salts, M is selected from the group of monovalent and divalent materials consisting of  $NH_4$ ,  $CH_3NH_3$ ,  $(CH_3)_2NH_2$ , Na, K, Ca, Zn, Mg, Cd, Ni, Fe, Co, Mo and Mn and n is equal to the valence of M.

35  $(CH_2)_2NH_2$

35 Na, K, Ca, Zn, Mg, Cd, Ni, Fe, Co, Mo and Mn and n is equal to the valence of M.

#### References Cited by the Examiner

##### UNITED STATES PATENTS

|    |           |         |                |       |          |
|----|-----------|---------|----------------|-------|----------|
| 40 | 2,589,209 | 3/1952  | Kardos         | ----- | 204-55 X |
|    | 2,740,754 | 4/1956  | Hoffman        | ----- | 204-55   |
|    | 2,860,089 | 11/1958 | Jackson        | ----- | 204-55   |
|    | 2,910,413 | 10/1959 | Strauss et al. | ----- | 204-55   |
|    | 2,966,448 | 12/1960 | Connor         | ----- | 204-55 X |
| 45 | 2,989,449 | 6/1961  | Mackey et al.  | ----- | 204-55   |
|    | 3,018,232 | 1/1962  | Bishoff et al. | ----- | 204-44   |

JOHN H. MACK, Primary Examiner.

JOHN R. SPECK, Examiner.

G. KAPLAN, Assistant Examiner.